

# United States Patent Office

3,026,242  
Patented Mar. 20, 1962

1

3,026,242

## COMPOSITION BOARD

John Robert Emery and Robert Morrow, Jr., Wilmington, Del., assignors to E. I. du Pont de Nemours and Company, Wilmington, Del., a corporation of Delaware  
No Drawing. Filed Aug. 6, 1957, Ser. No. 676,481  
4 Claims. (Cl. 162—146)

This invention relates to new products and more specifically to new composition boards reinforced with synthetic polymer filaments.

Composition boards conventionally contain cellulosic pulps which are beaten up with water and are formed into sheets or boards on cylinders or Fourdrinier machines. Such boards are frequently reinforced with resin binders which improve the stability, water resistance, and resistance to delamination of the products. While many varieties of pulp are used for different kinds of boards, it is customary, when high strength articles are desired, to use kraft pulp in place of cheaper but lower strength materials.

Among the uses of composition boards which require high strength material are shoe innersoles. In the construction of most shoes, the upper is stitched to the innersole and then the innersole is in turn stitched to the outersole. This construction puts a good deal of strain on the innersole material since the two rows of stitches are close to one another and are directed in opposite ways. There is a severe tearing force which is constantly exerted against the innersole material by these two rows of stitches and the stress is particularly great when the shoe is flexed as happens continually in normal walking. There is little or no abrasion stress exerted against innersoles, and the compressive forces are moderate, but the tensile stresses and stitch tensile stresses on shoe innersoles are extremely high and, when failure does occur, it is usually at the points of stitching. For this reason, materials of high stitch tensile strength are desired for use as shoe innersole. The most satisfactory such material is leather, but leather cannot be employed in high volume (low cost) shoe manufacturing operations because of the expense. For this reason, most shoe manufacturers employ kraft-pulp-based composition boards for shoe innersoles. However, even when the strongest kraft pulp is used, the rate of failure of composition innersoles has been undesirably high, particularly in shoes where the innersoles must be of light weight as, for example, in women's and children's shoes. Accordingly, woven fab-

2

great increase in cost. But even more important is that such materials should achieve the desired higher stitch tensile strength without the loss of other needed properties such as flexibility and resistance to delamination, and without necessitating laminating fabrics to the board.

It is an object of this invention to provide a new composition board suitable for use in shoe innersoles which has a high stitch tensile strength combined with the flexibility and resistance to delamination. It is another object of this invention to provide composition boards of high tensile strength and resistance to flex failure and impact failure. Another object of this invention is to provide composition boards containing synthetic organic polymer filaments which contribute to greater tensile strength and resistance to tearing and impact failure.

These objects are achieved in a composition board such as a shoe innersole, based on kraft pulp and containing between 3 and 10% by weight (based on total weight of pulp plus filaments) of high tenacity synthetic organic polymer filaments in the form of staple fibers at least  $\frac{1}{2}$  an inch long and not over 1 inch long and at least 10 denier per filament and preferably about 15 denier per filament, the composition board being bonded with a flexible elastomeric resin binder present to the extent of at least 18% and not over 25% of the total weight of the composition board.

Composition boards of the type specified can be prepared on conventional cylinder or Fourdrinier machines with no change in processing; in fact, because of the presence of the coarse synthetic fiber filaments, the board is easier to process than conventional boards because the water drains out more freely and rapidly and cuts down the cycle time for manufacture. The compositions within this invention are superior to conventional composition boards made without the synthetic organic fiber because they have a much higher stitch tensile strength and resistance to tearing without any sacrifice of other desirable physical properties, and these advantages can be achieved at only a modest increase in cost.

Examples of the practice of the present invention are summarized in Table I following. In these examples, boards are constructed on a cylinder machine using as furnish the mixture of fibers indicated in each case. The boards are tested for stitch tensile strength and examined for delamination by manual testing. A variety of formulations are illustrated and, as the table shows, compositions of the present invention offer a unique combination of advantages.

Table I

| Ex. | Composition                                                                             | Synthetic fiber DPF/<br>length, inches | Binder, <sup>1</sup><br>percent | Processing characteristics                                       | Characterization<br>of board  |                               |
|-----|-----------------------------------------------------------------------------------------|----------------------------------------|---------------------------------|------------------------------------------------------------------|-------------------------------|-------------------------------|
|     |                                                                                         |                                        |                                 |                                                                  | Stitch<br>tensile,<br>lb./pt. | Delamina-<br>tion<br>tendency |
| I   | Kraft, 50%; chrome leather scrap (control), 50%                                         |                                        | 15                              | Standard                                                         | .35                           | Low.                          |
| II  | Kraft, 50%; chrome leather scrap (control), 50%                                         |                                        | 20                              | do                                                               | .35                           | Low.                          |
| III | Kraft, 47%; chrome leather scrap, 50%; poly(hexamethylene adipamide) fiber, 3%          | 15%                                    | 20                              | Very high improved wet strength,<br>faster drainage on cylinder. | .70                           | Low.                          |
| IV  | Kraft, 45%; chrome leather scrap, 50%; poly(hexamethylene adipamide) fiber, 5%          | 15%                                    | 20                              | See Ex. III                                                      | .75                           | Low.                          |
| V   | Kraft, 45%; chrome leather scrap, 50%; poly(ethylene terephthalate) polyester fiber, 5% | 12%                                    | 20                              |                                                                  | .65                           | Low.                          |

<sup>1</sup> "Pliolite" 2001 latex resin (a flexible butadiene rubber based adhesive) manufactured by Goodyear Tire and Rubber Company.

rics are laminated to the thinner innersoles to improve stitch tensile strength.

It would be desirable to prepare a composition board of increased stitch tensile strength which could withstand successfully the great strains to which shoe innersoles are subjected. It would be, of course, most desirable that such a composition could be made without

70 Other synthetic fibers which are useful in this invention include high tenacity acrylic fibers such as polyacrylonitrile and copolymers containing at least about 85% bound acrylonitrile, high tenacity rayon, etc. In all cases, the stated high denier per filament fibers of the stated length are necessary.

While the examples show the preparation of composi-

tion boards using a specific latex resin, other flexible resins, based on latex, synthetic rubber formulations, neoprene and other elastomers are also satisfactory, provided that they bond the fibers of the composition as firmly as the resin exemplified.

As the examples show, the practice of the present invention gives a product with markedly improved physical properties at only a modest increase in cost. The practice of the present invention, however, is highly specific. It is not sufficient merely to add synthetic fiber filaments. The filaments must be present in a certain concentration range, and the filaments must be of a certain physical size. In addition, it is necessary that the resin content of the board be increased to offset the lower bonding tendency of the synthetic filaments of this invention. However, when all of these requirements are met, there is obtained a product which has superior physical properties and is highly useful as an article in manufacture.

While the examples of this invention have described the preparation of composition boards suitable for shoe innersoles, it is quite possible and practical to employ the same principles in the manufacture of other types of composition board. For example, tempered hard-board prepared from wood waste and bonded under high pressure and temperature with the lignins present in the bark of the wood waste is a well-known article of commerce. This composition board offers many attractive advantages for home construction, as a wall and ceiling surface, as a liner for closets and drawers and many other uses. The product is smooth, abrasion resistant and durable. However, it suffers from a lack of resistance to sudden impact. This undesired weakness can be overcome by the incorporation of 3 to 5% of heavy denier per filament synthetic organic fiber filaments as shown in Table I. When 3 to 5% of such filaments are added, the impact resistance of the board is greatly increased and other properties do not suffer. If too large a percentage of synthetic filament is added, the board does not bind satisfactorily. If low denier per filament

or short staple fibers are used, the inclusion of the organic filament does not contribute satisfactorily to the impact strength of the board. Similarly, the principle of the present invention can be applied in the manufacture of other types of composition board wherever a slight increase in cost can be tolerated for the achieving of substantially greater strength and its attendant advantages.

The claimed invention:

1. A composition board suitable for a shoe innersole comprising kraft pulp containing in admixture therewith, high tenacity synthetic organic polymeric fibers in the amount of from about 3% to about 10% based upon the weight of kraft pulp plus polymeric fibers, and having an average length between about  $\frac{1}{2}$  and about 1 inch and a denier per fiber of between about 10 and about 15, said composition board being bonded with a flexible elastomeric resin binder present in an amount between about 18% and about 25%, based upon the total weight of the composition board.
2. The composition board of claim 1 in which the fibers are polyethylene terephthalate.
3. The composition board of claim 1 in which the fibers are nylon.
4. The composition board of claim 3 in which the nylon is polyhexamethylene adipamide.

References Cited in the file of this patent

UNITED STATES PATENTS

|    |           |           |       |                |
|----|-----------|-----------|-------|----------------|
| 30 | 2,526,125 | Francis   | ----- | Oct. 17, 1950  |
|    | 2,653,870 | Kast      | ----- | Sept. 29, 1953 |
|    | 2,719,802 | Nottebohm | ----- | Oct. 4, 1955   |
|    | 2,723,935 | Rodman    | ----- | Nov. 15, 1955  |
| 35 | 2,777,787 | Bragg     | ----- | Jan. 15, 1957  |

FOREIGN PATENTS

|         |               |       |               |
|---------|---------------|-------|---------------|
| 674,577 | Great Britain | ----- | June 25, 1952 |
| 687,041 | Great Britain | ----- | Feb. 4, 1953  |
| 708,622 | Great Britain | ----- | May 5, 1954   |